

## UNITED STATES PATENT OFFICE.

HENRY H. SMITH, OF BERWYN, PENNSYLVANIA, ASSIGNOR OF ONE-HALF TO ANNA H. SMITH, OF BERWYN, PENNSYLVANIA.

## PROCESS OF MAKING BRONZE.

No Drawing.

Application filed December 11, 1923. Serial No. 680,039.

*To all whom it may concern:*

Be it known that I, HENRY H. SMITH, a citizen of the United States, residing at Berwyn, in the county of Chester and State 5 of Pennsylvania, have invented certain new and useful Improvements in Processes of Making Bronze, of which the following is a specification.

The object of my invention is to provide 10 a bronze of the non-granular type which will be more uniform in its physical properties and better adapted for bearings and to withstand pressure than the bronzes heretofore used, and the invention consists in the 15 method of manufacture hereinafter described.

In carrying out my invention I first fuse 20 approximately 40 parts in weight, of tin and 10 parts of zinc. To this molten alloy I add 1 part of phosphor copper thus forming 25 an alloy of tin, zinc and copper which will hereinafter be referred to as the foundation metal.

Approximately 306 parts of copper is then 25 fused and preferably raised to a temperature of 2200 degrees F. Then approximately 4 parts of boric acid are placed on top of the molten copper and, after a minute or two, the boric acid is stirred in, preferably with 30 a green wood pole. The foundation metal, either in molten state or in the form of ingots, is added to the molten copper and fused therewith thus forming the bronze.

In making the second and subsequent 35 heats, I prefer to fuse with the copper a part of the bronze produced by a previous heat which part may constitute about one third of the total. In other words, in the second and subsequent heats I fuse 51 parts 40 of foundation metal and about 178½ parts of previously made bronze with 306 parts of copper, 4 parts of boric acid being added as before. Addition of the previously made bronze does not change the proportions of 45 the ingredients but, due to the remelting and recrystallization of the metal, does produce a bronze of better resisting properties.

The resulting product is a bronze of greater uniformity and density than any 50 heretofore produced.

While I have described my invention as taking a particular form, it will be understood that the various parts may be changed without departing from the spirit thereof, 55 and hence I do not limit myself to the

precise construction set forth, but consider that I am at liberty to make such changes and alterations as fairly come within the scope of the appended claims.

Having thus described my invention, what I claim as new and desire to secure by Letters Patent is:—

1. A method of making bronze which consists in fusing approximately 40 parts tin, 10 parts zinc and 1 part phosphor copper to produce a foundation metal, fusing approximately 306 parts copper, raising the temperature of the copper to approximately 2200 degrees and fusing the foundation metal with the copper. 70

2. A method of making bronze which consists in fusing tin, zinc and phosphor copper to produce a foundation metal, fusing copper, adding boric acid to the copper and fusing the foundation metal with the copper. 75

3. A method of making bronze which consists in fusing tin, zinc and phosphor copper to produce a foundation metal, fusing copper, raising the temperature of the copper to approximately 2200 degrees, adding boric acid to the copper and fusing the foundation metal with the copper. 80

4. A method of making bronze which consists in fusing approximately 40 parts tin, 10 parts zinc and 1 part phosphor copper to produce a foundation metal, fusing approximately 306 parts copper, adding approximately 4 parts boric acid and fusing the foundation metal with the copper. 85

5. A method of making bronze which consists in fusing approximately 40 parts tin, 10 parts zinc and 1 part phosphor copper to produce a foundation metal, fusing approximately 306 parts copper, raising the temperature of the copper to approximately 2200 degrees, adding approximately 4 parts boric acid and fusing the foundation metal with the copper. 90

6. A method of making bronze which consists in fusing tin, zinc and phosphor copper to produce a foundation metal, fusing copper, and fusing the foundation metal and a portion of previously made bronze with the copper. 100

7. A method of making bronze which consists in fusing tin, zinc and phosphor copper to produce a foundation metal, fusing copper, adding boric acid to the copper, and fusing the foundation metal and a portion of previously made bronze with the copper. 105

70

75

80

85

90

95

100

105

110

8. A method of making bronze which consists in fusing approximately 40 parts tin, 10 parts zinc and 1 part phosphor copper to produce a foundation metal, fusing approximately 306 parts copper and fusing the foundation metal and approximately 178½ parts of previously made bronze with the copper.
9. A method of making bronze which consists in fusing approximately 40 parts tin, 10 parts zinc and 1 part phosphor copper to produce a foundation metal, fusing approx-

imately 306 parts copper, adding approximately 4 parts of boric acid to the molten copper, and fusing the foundation metal and approximately 178½ parts of previously made bronze with the copper. 15

In testimony whereof I have signed my name to this specification in the presence of two subscribing witnesses.

HENRY H. SMITH.

Witnesses:

MARY M. NORRIS,  
WANE MORAN.